# EUROPEAN PATENT SPECIFICATION

(11) **EP 0 452 405 B1**
(45) Date of publication and mention of the grant of the patent: **16.09.1992**
(21) Application number: 90902093.5
(22) Date of filing: 17.11.1989
(51) Int. Cl.: D01F 6/62, D01D 5/08

(54) **PROCESS FOR DIMENSIONALLY STABLE POLYESTER YARN**
VERFAHREN FÜR DIMENSIONELL STABILES POLYESTERGARN
PROCEDE POUR UN FIL POLYESTER INDEFORMABLE

(30) Priority: 03.01.1989 US 292864
(43) Date of publication of application: 23.10.1991
(73) Proprietor: AlliedSignal Inc., Morristown, New Jersey 07962-2245 (US)
(72) Inventor: HAMLYN, Maxwell, Charles, Cary, NC 27511 (US); LUCK, Thomas, Howard, Sanford, NC 27330 (US); NELSON, Charles, Jay, Chesterfield, VA 23236 (US)
(74) Representative: Lawrence, Peter Robin Broughton
(86) International application number: US8905081
(87) International publication number: WO9007592

(56) References cited:
- US-A- 4 101 525
- US-A- 4 491 657
- US-A- 4 690 866

## Description

### 1. Field of the Invention

This invention relates to a process for production of polyester multi-filament drawn yarn of 2.5 denier per filament (pf) (2.8 dtexpf) or greater, whereby high birefringence (Δn) yarns are prepared at lower spinning speeds and lower intrinsic viscosity than prior art processes.

### 2. Description of the Prior Art

Polyethylene terephthalate filaments of high strength are well known in the art and are commonly utilized in industrial applications including tire cord for rubber reinforcement, conveyor belts, seat belts, V-belts and hosing.

Dimensionally stable polyester (DSP) industrial yarns are desired to minimize sidewall indentations (SWI) in the bodies of radial tires and to achieve good tire handling characteristics. An additional objective is to make advanced DSP's having the strength and modulus equivalent to rayon at elevated tire service temperatures, while using up to 30 percent less material. While the current polyester tire cords have sufficient strength, their elevated temperature modulus is too low. U.S. Patent 4,101,525 to Davis et al. provides a high strength multifilament polyester yarn with low shrinkage and work-loss characteristics. While yarns exhibiting the features taught by Davis are classified as DSP's, they do not meet the modulus requirements for rayon replacement. Additionally, low denier per filament (dtexpf of 2.22 or less) and rapid cooling of the filament immediately after emerging from the spinneret can result in excessive filament breakage and thus yield yarn with poor mechanical quality. U.S. Patent 4,491,657 to Saito et al. discloses high modulus, low shrinkage polyester yarn, but requires a low terminal modulus to achieve good yarn to treated cord conversion efficiency for such dimensionally stable yarns. The low terminal modulus is translated into the treated cord and results in a lower tenacity than the high terminal modulus cords made by present invention. The process of Saito et al. requires high spinning speeds, which makes it difficult to incorporate the Saito process into a continuous spin-draw process, whereas the present invention permits the use of lower spinning speeds whereby more readily available and/or less costly equipment can be used.

U.S. 4,690,866 to Kumakowa et al. describes a means of making yarns which yield highly dimensionally stable treated cords using ultra high viscosity polymer. On a comparative experimental basis, i.e. utilizing our solvent system, the Kumakowa intrinsic viscosity (IV) values would be 5% higher than indicated in their patent, i.e. they require a minimum of 0.95 IV polymer by our measurements. Also, these cords have low terminal modulus and hence do not achieve the full tenacity benefit of a given polymer viscosity.

It is known, shown by the prior art cited above, that undrawn birefringence can be increased by increasing the spinning speed or yarn IV.

An important need exists for a process to produce high undrawn birefringence (Δnᵤ) yarns at lower spinning speeds and lower intrinsic viscosity (IV), than previously. Processing at lower speeds is important because of the speed limitations of commercial equipment, particularly winders. The ability to use lower IV means that costly processing steps such as solid state polymerization or costly/environmentally hazardous additives can be eliminated.

### Summary of the Invention

The invention relates to a process for production of a dimensionally stable drawn polyethylene terephthalate multifilament yarn having filaments of at least 2.5 denier per filament (2.8 dxpf) comprising the steps of:
a) extruding a polyethylene terephthalate polymer melt through a spinneret having a plurality of extrusion orifices to form filaments;
b) advancing the extruded multifilament yarn first through a delay zone then through a quenching zone to solidify the filaments in a controlled manner;
c) withdrawing the solidified multifilament yarn from the quenching zone at a desired spinning speed V;
   whereby steps a) through c) are performed under conditions to form a partially-oriented multifilament yarn having an undrawn birefringence (Δ nᵤ) of at least 0.020 and wherein Δ nᵤ = R_{f} V^{2.0} IV^{2.4} where IV is the intrinsic viscosity of the undrawn yarn and is at least 0.80 and R_{f}=RᵣRₑ is at least 9.0 x 10⁻³, Rr being a constant (O<Rᵣ<1) for given process conditions of steps a) and b), and Rₑ is at least 10.5 x 10⁻², Rₑ being the relationship D^{0.5}/Q^{0.7} (D=spinneret capillary diameter, in cm; Q=polymer flow rate through the capillary, in cm³/min/capillary); then
d) hot drawing the partially-oriented multifilament yarn. The process permits production of high undrawn birefringence yarns at lower speeds and lower IV's than previously demonstrated in the prior art.

### DESCRIPTION OF THE PREFERRED EMBODIMENT

The dimensionally stable polyester multifilament yarns made by the process of the present invention provide dimensionally stable treated cords when incorporated as fibrous reinforcement into rubber composites such as tires.

Dimensional stability is defined as high modulus at a given shrinkage and directly relates to tire sidewall indentations (SWI) and tire handling. While the modulus of the cord in the tire is the primary variable governing both SWI and handling, shrinkage is important in two ways. First, excessive cord shrinkage during tire curing can significantly reduce the modulus from that of the starting treated cord. Second, cord shrinkage is a potential source of tire non-uniformity. Thus, comparison of modulus and tenacity at a given shrinkage is a meaningful comparison for tire cords. Since tire cords experience deformations of a few percent during service, a good practical measure of modulus is LASE-5 (load at 5 percent elongation). Alternatively, E_{4.5} (elongation at 4.5 g/d load (4.0 cN/dtex)) can be used as a practical measure of compliance.

For both tire SWI and handling, modulus at elevated temperature (up to 110°C) is the important parameter governing performance. Due to the highly crystalline nature of treated cords based on conventional or dimensionally stable tire yarns, the modulus retention (in percent) at elevated tire temperatures is essentially similar for all current commercial treated cords and for those of this invention when loss modulus peaks occur at 110°C or greater. Thus, room temperature measurement of LASE-5 is sufficient to establish meaningful differences in polyester cord dimensional stability.

The polyester yarn contains at least 90 mol percent polyethylene terephthalate (PET). In a preferred embodiment, the polyester is substantially all polyethylene terephthalate. Alternatively, the polyester may incorporate as copolymer units minor amounts of units derived from one or more ester-forming ingredients other than ethylene glycol and terephthalic acid or its derivatives. Illustrative examples of other ester forming ingredients which may be copolymerized with the polyethylene terephthalate units include glycols such as diethylene glycol, trimethylene glycol, tetramethylene glycol, hexamethylene glycol, etc., and dicarboxylic acids such as isophthalic acid, hexahydroterephthalic acid, bibenzoic acid, adipic acid, sebacic acid, azelaic acid, etc.

The polymer may be polymerized in a separate operation or polymerized in a directly coupled continuous polymerization and direct melt spinning process.

An important aspect of this invention permits obtaining high undrawn birefringence yarn without the need to utilize molecular weight enhancing additives such as multifunctional coupling agents exemplified by 2,2′-bis(2-oxazoline). Catalysts for the polymerization reaction are not considered to be included in the definition of molecular weight enhancing additive.

The multifilament yarn of the present invention commonly possesses a denier per filament of about 2.5 to 20 (e.g. about 3 to 10) (about 2.8 to 22, e.g. about 3.3 to 11 dtexpf), and commonly consists of about 6 to 600 continuous filaments (e.g. about 20 to 400 continuous filaments). The denier per filament (texpf) and the number of continuous filaments present in the yarn may be varied widely within the ranges of this invention as will be apparent to those skilled in the art.

The multifilament yarn made by the process is particularly suited for use in industrial applications including rubber composites, ropes, cordage and tarps. The fibers are particularly suited for use in environments where elevated temperatures (e.g. 80°C to 110°C) are encountered.

The yarn characterization parameters referred to herein may conveniently be determined by testing the multifilament yarn which consists of substantially parallel filaments.

Undrawn birefringence (Δnᵤ) was determined using a polarizing light microscope equipped with a Berek compensator.

Intrinsic viscosity (IV) of the polymer and yarn is a convenient measure of the degree of polymerization and molecular weight. IV is determined by measurement of relative solution viscosity (ηᵣ) of PET sample in a mixture of phenol and tetrachloroethane (60/40 by weight) solvents. The relative solution viscosity (ηᵣ) is the ratio of the flow time of a PET/solvent solution to the flow time of pure solvent through a standard capillary. Billmeyer approximation (J. Polym. Sci. 4, 83-86 (1949)) is used to calculate IV according to$\text{IV = .25} \frac{{\text{(η}}_{\text{r}} \text{-1)}}{\text{C}} \text{+ .75} \frac{{\text{1nη}}_{\text{r}}}{\text{C}}$
where C is concentration in gm/100 ml. In this study, the concentration was 1.3 gms/100 ml. It will be understood that IV is expressed in units of deciliters per gram (dl/g), even when such units are not indicated. Comparison to IV measurements in other solvents is given in an article by C. J. Nelson and N. L. Hergenrother, J. Poly. Sci., 12 2905 (1974). The invention makes possible obtaining high modulus drawn yarn without the need to utilize exceptionally high IV polymer. Satisfactory drawn yarns with high Δ nᵤ with IV of at least 0.80, for example 0.85 to 0.95 can be obtained by this invention.

The tensile properties referred to herein were determined on yarns conditioned for two hours through the utilization of an Instron tensile tester (Model TM) using a 10-inch (25.4 cm) gauge length and a strain rate of 120 percent per minute in accordance with ASTM D885. All tensile measurements were made at room temperature.

Elongation at the specified load of 4.5 g/d (E_{4.5}) (4.0cN/dtex) is inversely related to modulus. It is particularly useful in that the sum E_{4.5} + FS (FS = fire shrinkage) is a good indicator of dimensional stability for yarns processed under different relaxation levels. Lower sums (E_{4.5} + FS) indicate better dimensional stability. The drawn yarn of the present invention is produced with Δnᵤ greater than 0.020 and posses a dimensional stability defined by E4.5 + FS < 16%. Free shrinkage (FS) values were determined in accordance with ASTM D885 with the exception that the testing load was 0.009 g/d (0.008 cN/dtex). Such improved dimensional stability is of particular importance if the product serves as fibrous reinforcement in a radial tire.

Identified hereafter is a description of the continuous spin-draw process which has been found to be capable of forming the desired improved yarns. Figures 1 and 2 illustrate apparatus which may be utilized to practice the process of this invention, though it will be recognized by those of skilled in the art that the apparatus illustrated may be modified in known ways.

Referring to Figs. 1 and 2, like numbers indicate like apparatus. Molten polymer is fed by extruder 11 to spin pump 12 which feeds spin block 13 containing a spinneret and a spinning filter disposed between the spin pump and spinneret. The spinneret is designed for the extrusion of one or more ends of filaments, each end containing a plurality of filaments. Fig. 1 illustrates the simultaneous extrusion of two ends 14 and 15 of multifilament, continuous filament yarn from one spinneret. Ends 14 and 15 are extruded from the spinneret at a spinning temperature in the range of 282 to 320°C and at a desired polymer volumetric flowrate (Q, cm³/min/capillary), and are passed downwardly from the spinneret into a delay zone, chamber 16, which preferably is a quiescent delay zone or a heated sleeve of a desired delay length preferably 1 to 40 inches (2.5 to 102 cm), maintained at a desired heated sleeve temperature preferably 100 to 450°C. Yarn leaving chamber 16 is passed directly into the top of the quenching zone, apparatus 17, preferably a radial inflow quench. The quench chamber is an elongated chimney of conventional length for example 1 to 40 inches (2.5 to 102 cm). Ends 14 and 15 of yarn are lubricated by finish applicator 18. A spinning finish composition is used to lubricate the filaments. For the examples in this application, finish applicator 18 was a lube roll which is rotated with the direction of the yarn movement. Other means of applying finish could also be used.

To achieve desired properties in the final drawn yarn, it is necessary to hot draw the partially-oriented multifilament yarn withdrawn from the quenching zone, for example to at least 85 percent of the maximum draw ratio. This can be accomplished either in an off-line drawing process or preferably in a continuous spin-draw process. The drawing may be multiple steps and include high temperature annealing with or without relaxation. In this illustration, ends 14 and 15 are then transported to spin draw panel 21. A typical configuration is shown in Fig. 2. In Fig. 2, ends 14 and 15 are all processed on the same single set of forwarding (first roll 1), drawing (rolls 2-3 and rolls 5-6) and relaxing rolls (rolls 7-8). From draw roll 2, the ends are passed through a steam impinging draw point localizing steam jet 4. From relaxing rolls 7 and 8, the yarn ends are forwarded to winder 22. For the discussion following V is taken as the linear speed of roll 1.

With respect to conditions for operating the apparatus to achieve the process of this invention, it is generally known that undrawn birefringence (Δ nᵤ) can be increased by increasing the spinning speed (V given in km/min) or the IV of the yarn (dl/g). By experimental work accomplished during the course of this invention, this can now be quantified by the following experimentally determined relationship:${\text{Δ n}}_{\text{u}} {\text{= R}}_{\text{f}} {\text{V}}^{\text{2.0}} {\text{IV}}^{\text{2.4}}$

V is the spinning speed given in kilometers/ minute. IV is the intrinsic viscosity of the undrawn yarn given in dl/g. R_{f} is a value characteristic of the additional processing variables other than V and IV.

For conventional and prior art processes, R_{f} is typically < 8 x 10⁻³, whereas for the process of this invention R_{f} is > 9.0 x 10⁻³. Of course, the higher the R_{f} value, the higher the undrawn birefringence for a given IV and V. Apparently, the combination of high molecular weight (IV > 0.80) and inherent stiffness of the PET molecule results in a sufficiently slow relaxation rate in the molten state to achieve high R_{f} values. High R_{f} values, for example R_{f} ≧ 15 x 10⁻³, are readily attainable by this invention and are of prime commercial interest.

R_{f} can be broken down into two more basic terms:${\text{R}}_{\text{f}} {\text{= R}}_{\text{r}} {\text{R}}_{\text{e}}$
wherein Rᵣ has a value which is related to the retention in orientation after thermally induced polymer relaxation with the constraint that O<Rᵣ<1. This parameter increases with increasing severity of the quenching and decreases with increasing extruded polymer temperature and heated sleeve length and temperature. One skilled in the art can adjust these parameters to maximize Δ nᵤ and still maintain good spinnability.

The core of the invention is in the Rₑ term which is related to the effective polymer extension from flow orientation in the spinneret and draw-down in the spin column. The net result is substantial orientation even at moderate spinning speeds. The experimentally determined relationship is${\text{R}}_{\text{e}} \text{=} \frac{{\text{D}}^{\text{0.5}}}{{\text{Q}}^{\text{0.7}}}$
where D is the spinneret capillary diameter (inches) and Q is the polymer flow rate through the capillary expressed in cm³/min/capillary. Q is calculated using a polymer density of 1.2 gm/cm³. This invention also teaches the proper combination of D and Q to achieve Rₑ of at least 10.5 x 10⁻². More preferred, Rₑ is at least 13 x 10⁻².

If one looks only at the IV range 0.80-0.95, a simplified expression may be obtained which shows the advantage of this invention over prior art, with Δ nᵤ of at least 7.0 x 10⁻³ V². It may be preferred to achieve even higher birefringence for a given V, with Δ n^{u} of at least 11.5 x 10⁻³ V². Thus, for this viscosity range, the invention can also be defined solely in terms of V.

The particular examples which follow show how proper selection of process variables results in R_{f} ≧ 9.0 x 10⁻³ and the desired improved yarns which exhibit improved dimensional stability. The comparative examples are taken from the patents previously cited and are summarized in Table I. This table contains all examples in which (a) the drawn yarn had a dpf of at least 2.5 (2.8 dxpf), (b)Δnᵤ was at least 0.020, and (c) the yarn IV was between 0.85 and 0.96. The latter IV range was chosen since it is close to the 0.88 - 0.92 range in our examples.

### EXAMPLE 1

PET polymer was pumped at 296°C to a spinneret containing multiple orifices, each orifice being of 0.030 inch (0.076 cm) diameter (D=0.030 inch). The extension rate per hole (Q) was 0.88 cm³/min. The filaments were passed through a 1 inch (2.54 cm) heated sleeve and then quenched in a radial quench stack. The spun yarn was subsequently drawn on a panel similar to figure 2, with roll 1 maintained at 90°C, the yarn drawn 1.5/1 to unheated rolls 2, 3 with a normal ambient temperature of 40-50°C, then drawn 1.6/1 from rolls 2, 3 to rolls 5, 6 maintained at 200°C, the yarn was then relaxed to rolls 7, 8 at 1 to 1.5 percent. Rolls 7 and 8 had an operating temperature of 150°C. The drawn yarn was taken up at 2.98 km/min. Polymer thruput for the two ends was 85 Ibs./hour (39 kg/hour). The drawn yarn was 1004 denier (1114 dtex), 3.3 dpf (3.7 texpf), 17.5 lbs. breaking strength (77.8N), 7.9 g/d tenacity (7.0 cN/dtex) , 10.6 percent ultimate elongation, 3.9 g/d LASE-5 (3.44 cN/dtex), 5.5% E_{4.5} and 9.2 percent FS. The sum E_{4.5} + FS is 14 percent. The undrawn yarn birefringence (Δ nᵤ) was 0.026 and IV was 0.92 dl/g. R_{f} was 24 x 10⁻³. The yarn produced in this example, while produced at a moderate spinning take-up speed usually associated with standard yarn products, is then shown to have that enhanced dimensional stability associated with substantially higher spinning speeds in the prior art. R_{f} and Rₑ were 24 x 10⁻³ and 19 x 10⁻², respectively.

### EXAMPLE 2

An ultradimensionally stabilized PET was produced in the following manner. PET polymer was pumped into a spinneret containing multiple orifices, each orifice being of 0.027 inch (0.069 cm) diameter (D = 0.027 inch). Q was 1.3 cm³/min/cap. The filaments were then passed through a heated sleeve (HST = 220-300°C, residence time 0.02-0.03 sec) and quenched in a radial quench stack. The spun yarn was first drawn 1.4/1 between rolls at 90°C and unheated rolls, then drawn 1.15/1 between these and rolls maintained at 220°C. The drawn yarn was then relaxed at 3% to rolls maintained at 135°C. The yarn was taken up by a high speed winder at 4.60 km/min. The drawn yarn was 924 denier (1026 dtex), 3.3 dpf (3.7 texpf), 5.8 g/d tenacity (5.1 cN/dtex), 4.1 g/d LASE-5 (3.6 cN/dtex), 6.5 percent E_{4.5}, 10.3 percent ultimate elongation, 4.3 percent free shrinkage. The sum E_{4.5}, + FS was 10.8 percent. The undrawn yarn birefringence was 0.082 and IV was 0.92 dl/g. R_{f} was 11 x 10⁻³ and Rₑ was 14 x 10⁻².

### EXAMPLE 3

Yarn (IV = 0.92) was produced in a similar manner to that in Example 1, only (a) a 2-inch (5cm) sleeve was heated to 220-300°C (b) the spinneret orifice was 0.018 inch (0.046 cm), and (c) Q was 1.0 cm³/min/cap. The drawn yarn was taken-up at 4.72 km/mins after experiencing a 2.46/1 hot draw ratio. This yarn had similar properties to Example I: 3.3 dpf (3.7 dtexpf), tenacity of 8.1 g/d (7.15 cN/dtex), ultimate elongation of 10.0%, LASE-5 of 3.9 g/d (3.44 cN/dtex), E_{4.5} of 5.5%, and free shrinkage of 10.0%. The 0.028 undrawn birefringence corresponded to a R_{f} of 11 x 10⁻³. Rₑ was 13 x 10⁻².

### EXAMPLE 4

A high viscosity yarn (IV = 0.88) was prepared similar to Example 2, only:D = 0.018 inches (0.046 cm) and V = 3.5 km/min. The undrawn yarn had a birefringence of 0.088 which corresponds to R_{f} = 9.8 x 10⁻³. Drawn dpf was 2.7 (3.0 dtexpf) and Rₑ was 11 x 10⁻².

## Claims

1. A process for the production of a dimensionally stable drawn polyethylene terephthalate multifilament yarn having filaments of at least 2.5 denier per filament (2.8 dtexpf) comprising the steps of:
a) extruding a polyethylene terephthalate polymer melt through a spinnerette having a plurality of extrusion orifices to form filaments;
b) advancing the extruded multifilament yarn first through a delay zone then through a quenching zone to solidify the filaments in a controlled manner;
c) withdrawing the solidified multifilament yarn from the quenching zone at a desired spinning speed V (km/min);
whereby steps a) through c) are performed under conditions to form a partially-oriented multifilament yarn having an undrawn birefringence ( Δ nᵤ) of at least 0.020 and wherein Δ nᵤ = R_{f} V²^{.0} IV²^{.4} where IV is the intrinsic viscosity of the undrawn yarn and is at least 0.80 and R_{f}=RᵣRₑ is at least 9.0 x 10⁻³, Rr being a constant (O<Rᵣ<1) for given process conditions of steps a) and b), and Rₑ is at least 10.5 x 10⁻², Rₑ being the relationship D^{0.5}/Q^{0.7} (D = spinneret capillary diameter, in cm; Q=polymer flow rate through the capillary, in cm³/min/capillary); then
d) hot drawing the partially-oriented multifilament yarn.

2. The process of claim 1 wherein R_{f} is at least 15 X 10⁻³.

3. The process of claim 1 wherein Rₑ is at least 13 X 10⁻².

4. The process of claim 1 wherein IV is 0.80 to 0.95 and Δ nᵤ is at least 7.0 x 10⁻³ V².

5. The process of claim 1 wherein Δ nᵤ is at least 11.5 x 10⁻³ V².

6. The process of claim 1 wherein IV is at least 0.85.

7. The process of claim 1 wherein the diameter D of said extrusion orifices is at least 0.027 inches (0.069 cm).

8. The process of claim 1 additionally comprising the step of polymerizing said polyethylene terephthalate polymer, thereby having a continuous polymerization and direct melt spinning process.

9. The process of claim 1 or claim 8 wherein said polyethylene terephthalate polymer is polymerized in the absence of a molecular weight enhancing additive.

## Patentansprüche

1. Verfahren zum Herstellen eines dimensionell stabilen, gestreckten Polyäthylen-Terephthalat-Garnes aus einem Multifilament mit Fasern von wenigstens 2,5 Denier pro Filament (2,8 dtexpf) mit den folgenden Verfahrensschritten:
a) Extrudieren einer Polyäthylen-Terephthalat-Polymerschmelze durch eine Spinndüse mit einer Vielzahl von Extrusionsöffnungen für die Bildung von Fasern;
b) Vorwärtsbewegen des extrudierten Multifilament-Garnes zuerst durch eine Aufenthaltszone, und dann durch eine Kühlzone, um die Fasern in kontrollierter Weise zu verfestigen;
c) Abziehen des verfestigten Multifilament-Garnes aus der Kühlzone mit gewünschter Spinngeschindigkeit V (km/min);
wobei die Verfahrensschritte a) bis c) unter Bedingungen zum Bilden eines teilweise orientierten.Multifilament-Garnes mit einer ungestreckten Doppelbrechung (Delta nᵤ) von wenigstens 0,020 durchgeführt werden, wobei${\text{Delta n}}_{\text{u}} {\text{= R}}_{\text{f}} {\text{V}}^{\text{2.0}} {\text{IV²}}^{\text{.4}} \text{,}$ worin IV die Strukturviskosität des ungestreckten Garnes ist und zumindest 0,80 beträgt, und R_{f}=RᵣRₑ wenigstens 9.0 X 10⁻³ beträgt, Rr eine Konstante (0<Rᵣ<1) für gegebene Verfahrensbedingungen der Verfahrensschritte a) und b) ist, und Rₑ wenigstens 10,5 x 10⁻² beträgt, wobei Rₑ das Verhältnis D^{0,5}/Q^{0,7} (D=Kapillardurchmesser der Spinndüse in cm; Q=die Durchflußleistung an Polymer durch die Kapillaren in cm³/min/Kapillare) bezeichnet; dann
d) Heißverstrecken des teilweise orientierten Multifilament-Garnes.

2. Verfahren nach Anspruch 1, worin R_{f} zumindest 15 x 10⁻³ beträgt.

3. Verfahren nach Anspruch 1, worin Rₑ zumindest 13 x 10⁻² beträgt.

4. Verfahren nach Anspruch 1, worin IV 0,80 bis 0,95 und Delta nᵤ zumindest 7,0 x 10⁻³ V² beträgt.

5. Verfahren nach Anspruch 1, worin Delta nᵤ zumindest 11,5,0 x 10⁻³ V² beträgt.

6. Verfahren nach Anspruch 1, worin IV zumindest 0,85 beträgt.

7. Verfahren nach Anspruch 1, worin der Durchmesser D der Extrusionsöffnungen zumindest 0,027 Zoll (0,069 cm) beträgt.

8. Verfahren nach Anspruch 1, das zusätzlich den Verfahrensschritt des Polymerisierens des Polyäthylen-Terephthalat-Polymers mit einer kontinuierlichen Polymerisation und einem direkten Schmelzverspinnungsverfahren aufweist.

9. Verfahren nach Anspruch 1 oder 8, worin das Polyäthylen-Terephthalat-Polymer in Abwesenheit eines das Molekulargewicht vergrößernden Zusatzes polymerisiert wird.

## Revendications

1 - Procédé pour la fabrication d'un fil à multifilaments en polytéréphtalate d'éthylène étiré, dimensionnellement stable, ayant des filaments d'au moins 2,5 deniers par filament (2,8 dtexpf) comprenant les étapes consistant à :
a) extruder une masse fondue d'un polymère de polytéréphtalate d'éthylène dans une filière comportant une multitude d'orifices d'extrusion afin de former des filaments;
b) faire avancer le fil extrudé à multifilaments tout d'abord dans une zone à retard, puis dans une zone de refroidissement de manière à solidifier les filaments de façon contrôlée;
c) extraire le fil solidifié à multifilaments de la zone de refroidissement à une vitesse de filage V désirée (km/min);
d'où il résulte que les étapes a) à c) sont exécutées dans des conditions permettant de former un fil à multifilaments partiellement orienté, ayant une biréfringence à l'état non étiré (Δnᵤ) d'au moins 0,020 et dans lequel Δnᵤ = R_{f} V²^{,0} IV²^{,4}, où IV est la viscosité intrinsèque du fil non étiré et est au moins égal à 0,80 et R_{f}=RᵣRₑ est d'au moins 9,0 x 10⁻³, Rr étant une constante (0<Rᵣ<1) pour des conditions de traitement données dans les étapes a) et b), et Re est au moins 10,5 x 10⁻², Re étant la relation D⁰^{,5}/Q^{0,7} (D = diamètre du capillaire de la filière, en cm; Q = débit du polymère dans le capillaire, en cm³/min/capillaire); puis
d) étirer à chaud le fil à multifilaments partiellement orienté.

2 - Procédé selon la revendication 1, dans lequel R_{f} est égal à au moins 15 x 10⁻³.

3 - Procédé selon la revendication 1, dans lequel Rₑ est égal à au moins 14 x 10⁻².

4 - Procédé selon la revendication 1, dans lequel IV est égal à 0,80-0,95 et Δnᵤ est égal à au moins 7,0 x 10⁻³ V².

5 - Procédé selon la revendication 1, dans lequel Δnᵤ est égal à au moins 11,5 x 10⁻³ V².

6 - Procédé selon la revendication 1, dans lequel IV est égal à au moins 0,85.

7 - Procédé selon la revendication 1, dans lequel le diamètre D desdits orifices d'extrusion est égal à au moins 0,069 cm.

8 - Procédé selon la revendication 1, comprenant en outre l'étape de polymérisation dudit polymère de polytéréphtalate d'éthylène, d'où il résulte qu'on a un procédé de polymérisation en continu et de filage direct d'une masse fondue.

9 - Procédé selon la revendication 1 ou la revendication 8, dans lequel ledit polymère de polytéréphtalate d'éthylène est polymérisé en l'absence d'un additif d'amélioration de la masse moléculaire.
